

## UNITED STATES PATENT OFFICE

HENRY W. BOTTS, OF KENVIL, AND HUBERT H. CHAMPNEY, OF SUCCASUNNA, NEW JERSEY, ASSIGNORS TO HERCULES POWDER COMPANY, OF WILMINGTON, DELAWARE, A CORPORATION OF DELAWARE

## EXPLOSIVE

No Drawing.

Application filed January 24, 1930. Serial No. 423,259.

This invention relates to an improvement in explosives and more particularly to an improved explosive gelatin.

Heretofore explosive gelatin has been known to possess a material advantage in that it is water resistant and hence may be effectively used in the presence of water, as in wet bore holes. However, explosive gelatin is of high density and brisance and hence renders it undesirable for any general use and rendering it distinctly disadvantageous for many purposes where its use is necessitated by the presence of water. Thus, for example, in the blasting of easily shatterable material, where shattering is undesirable, explosive gelatin is distinctly objectionable as an explosive, though its use in such materials is frequently necessitated due to the presence of water in bore holes.

Now, in accordance with this invention, an improved explosive is made available which will be found to be highly water resistant, as is explosive gelatin and, at the same time, of substantially less density and brisance than is explosive gelatin, and hence will be highly efficient for use in the blasting of shatterable material in the presence of water.

The explosive in accordance with this invention comprises as essential ingredients ammonium nitrate in major proportion, carbonaceous material, which may be, for example, oat hulls, bagasse, starch, ivory meal, or the like, or mixtures thereof, nitrocotton, and nitroglycerin.

As will be understood the explosive oil acts to gelatinize the nitrocotton, and render the explosive as a whole gelatinous and water resistant.

In many cases an oxidizing salt, as sodium nitrate, will be included and it will be understood that the nitroglycerin may be admixed with nitrosugar, nitroglycol, tetranitroglycerin, or the like. Further, dinitrotoluene may desirably be included and will be in-

cluded when a mixture of nitroglycerin and tetranitroglycerin is used.

The carbonaceous content of the explosive is desirably, at least in part, composed of material which is of low density and of low absorptive capacity in the explosive oil.

The various ingredients may be incorporated in the explosive in varying proportions it, however, being essential that the ammonium nitrate be used in amount not less than 50% 50%, though it may be used in amounts up to 80% and that sufficient explosive oil, as nitroglycerin, be used to gelatinize the nitrocotton used and to render the explosive water resistant as a whole.

As illustrative of the ranges within which the various ingredients of the explosive respectively may be used, attention is called, for example, to the following table:

Table A

|                                                                                         | Per cent |
|-----------------------------------------------------------------------------------------|----------|
| Nitroglycerin                                                                           | 15-26    |
| Nitrotoluene (if included)                                                              | Up to 6  |
| Nitrocotton                                                                             | 0.1-0.35 |
| Ammonium nitrate                                                                        | 50-80    |
| Sodium nitrate (if included)                                                            | Up to 20 |
| Carbonaceous material (for example, oat hulls, ivory meal, bagasse, starch or mixtures) | 4-14     |

It will be understood that the explosive embodying this invention will be of substantially less density than explosive gelatin and as a consequence will be capable of a substantially greater cartridge count than is possible with explosive gelatin. Thus, with this improved explosive cartridge counts substantially in excess of 100 standard 11/4" x 8" cartridges per fifty pounds of explosive may be obtained as compared with 100 standard cartridges per fifty pounds of explosive heretofore obtainable as a maximum with explosive gelatin.

An explosive embodying this invention, which will be highly water resistant will have

a cartridge count of 120 standard  $1\frac{1}{4}$ " x 8" cartridges per fifty pounds of explosive, and will have desirable brisance, may be, for example, composed as shown in the following table:

|    | <i>Table B</i>   | Per cent |
|----|------------------|----------|
|    | Nitroglycerin    | 17       |
|    | Nitrotoluene     | 3        |
|    | Nitrocotton      | 0.2      |
| 10 | Ammonium nitrate | 64.8     |
|    | Sodium nitrate   | 8.0      |
|    | Oat hulls        | 2.0      |
|    | Ivory meal       | 5.0      |

15 The explosive in accordance with this invention may be mixed in any suitable manner, as for example, the explosive oil and nitrocotton may be gelatinized and the other ingredients added, though if desirable the ingredients may be mixed in other order and, 20 it will be understood that no special form of apparatus is required for the mixing. The explosive, while gelatinized, will be found to be only slightly sticky and may be cartridgeed, 25 for example, in the usual dynamite packing machines.

It will now be noted that in accordance with this invention a novel explosive is provided which will have the desirable water resistance 30 of explosive gelatin, may be readily produced and cartridgeed, and at the same time will be of a desirable density and brisance for blasting under conditions where the use of explosive gelatin is dictated due to the presence of 35 water, but where the high density and brisance of explosive gelatin is highly disadvantageous.

What we claim and desire to protect by Letters Patent is:

40 1. An improved explosive including the following ingredients in about the following proportions:

|    | Per cent         |      |
|----|------------------|------|
|    | Nitroglycerin    | 17.0 |
|    | Nitrotoluene     | 3.0  |
| 45 | Nitrocotton      | 0.2  |
|    | Ammonium nitrate | 64.8 |
|    | Sodium nitrate   | 8.0  |
|    | Oat hulls        | 2.0  |
|    | Ivory meal       | 5.0  |

50 2. An improved plastic explosive including as ingredients explosive oil and nitrocellulose in amounts respectively in about the proportion 20:0.2, ammonium nitrate in excess of 55 50% and substantially non-absorbent carbonaceous material.

3. An improved plastic explosive including the following ingredients in about the following proportions: nitroglycerine 17.0%, nitrotoluene 3.0%, nitrocotton 0.2%, ammonium nitrate in excess of 50% and substantially non-absorbent carbonaceous material.

4. An improved explosive including explosive oil about 20%, nitrocellulose about 0.2%, 60 ammonium nitrate in excess of 50% and sub-

stantially non-absorbent carbonaceous material.

In testimony of which invention, we have hereunto set our hands, at Kenvil, N. J., on this 21st day of January, 1930.

HENRY W. BOTTs.  
HUBERT H. CHAMPNEY.

70

75

80

85

90

95

100

105

110

115

120

125

130

135